

## UNITED STATES PATENT OFFICE.

DANIEL GRAY AND RICHARD O. BAILEY, OF ONEIDA, AND WILLIAM S. MURRAY, OF UTICA, NEW YORK, ASSIGNORS TO ONEIDA COMMUNITY, LIMITED, OF ONEIDA, NEW YORK, A CORPORATION OF NEW YORK.

TARNISH-RESISTING SILVER AND SILVER PLATE AND PROCESSES FOR PRODUCING THE SAME.

No Drawing. Application filed April 3, 1924, Serial No. 703,974. Renewed December 13, 1928.

This invention relates to tarnish resisting silver, silver alloys and silver plated ware, and to a process of producing the same.

The tarnishing of silver, silver alloy or silverplated articles on the shelves of the dealer, and in the house and other places of use, is a source of much inconvenience and expense in that frequent cleaning of the articles, by rubbing, polishing, etc. is necessary to restore them to their natural color and brightness, such cleaning also impairing the original lustre or finish and in time resulting in more or less wear of the polished surface and its surface ornamentation.

It is the object of this invention to overcome these objections by providing silver, silver alloy and silverplated ware which will be tarnish resisting, and also a process of producing such ware.

This is accomplished according to the present invention by combining with the silver, silver alloy or silver plate a metal or metals which, in such combination, will have a shielding action as to tarnish so that the article as a whole will be tarnish resisting.

The metal selected for this purpose is mercury.

The present invention has particular reference to the production of silver, silver alloy or silver plate, to all of which mercury has been added.

According to the present invention this tarnish resisting silver, silver alloy and silver plate are produced by the use of mercury, as before stated. The silver, silver alloy or silver plate is exposed to the vapor of mercury in an oven maintained at a suitable temperature for vaporizing the mercury, and under this condition the mercury is absorbed by the silver, silver alloy or silver plate.

One detailed way of carrying out the process may be described as follows:—

The silver, silver alloy or silver plate is

placed in a steam jacketed oven of about 1 cubic foot capacity together with an excess 45 of mercury. We have found that temperatures ranging from 290° F. to 315° F. are suitable for the purposes of this process. The mercury is contained in shallow open dishes. The time of exposure which we use 50 ranges from a few minutes to a few hours, depending upon the amount of mercury which we wish to be absorbed by the silver, silver alloy or silver plate.

Depending upon the amount and surface 55 of silver, silver alloy or silver plate to be treated, varying percentages of mercury may be added.

Very good results have been obtained in this respect by the absorption by the silver, 60 silver alloy or silver plate of from fractional percentages up to as high as 14% of its weight of mercury.

What is claimed is:

1. The herein-described process of producing tarnish-resisting silver, silver alloy or silverplate which consists in exposing the silver, silver alloy or silverplate to mercury in an oven maintained at a suitable temperature for the vaporization of the mercury and 70 the absorption thereof by the silver, silver alloy or silverplate.

2. An article having a working surface containing not less than about 90% of silver and a quantity of mercury sufficient to render said 75 surface resistant to tarnish, but not sufficient to form a soft amalgam with said silver.

In testimony whereof, we have hereunto set our hands.

DANIEL GRAY.  
RICHARD O. BAILEY.  
WILLIAM S. MURRAY.